

## UNITED STATES PATENT OFFICE

2,369,613

## DYEING AND FINISHING OF TEXTILES

Ernst Schubert, Jonsdorf, near Zittau, and Heinz Pierer, Zittau, Germany; vested in the Alien Property Custodian

No Drawing. Application October 24, 1941, Serial No. 416,423. In Yugoslavia January 10, 1941

1 Claim. (Cl. 8—18)

The present invention relates to a method of simultaneously dyeing and finishing textile materials whereby a series of valuable effects is attained.

To obtain ordinary effects, as for instance proofness against creasing, a slight shrinkage or also to ensure a proofness against swelling, to attain a matte surface or the like, it is well known to finish textile materials by means of phenol-aldehyde artificial resins or urea-aldehyde artificial resins by soaking or impregnating the fabric with a solution containing artificial resins or products of artificial resins, wherein aqueous solutions are used. The operation may also be carried out by applying to the fiber, components which will form a resin. The impregnated fabric is then subjected to a heat treatment and thereby the artificial resins are either hardened or initially formed upon the fibre.

These finishing methods are carried out as final methods and hitherto were applied in connection with dyed fabric only after termination of the dyeing method. Only a limited number of genuine dye-stuffs was available for dyeing textile materials which later were to be subjected to an artificial resin finishing treatment.

Now, according to the present invention a method is proposed which permits carrying out simultaneously, in one and the same operation, a dyeing and a finishing method by means of artificial resins by applying the dyestuff and the artificial resin to the fibre by a single bath, wherewith in some cases the fabric is previously treated with a salt which can combine with a component for forming the dye-stuff which is applied to the fibre by the same bath as the artificial resin. This method has the advantage that dyeing effects of substantially better properties, for instance with regard to genuineness, are obtained without interfering with the desired finishing effects.

In accordance with the preferred embodiment of the invention, the textile material is impregnated in a dye bath which contains water-soluble components for forming a resin, or a water-soluble preliminary product, for instance dimethylol urea, as well as a catalyst for forming a resin and/or a hardening catalyst as well as a desired dye-stuff. Such artificial resins, preliminary products of artificial resins and components for forming artificial resin may be used which are soluble in the aqueous solution of the catalyst and which are capable of hardening to form the final resin when heated. For instance, if alkali is used as catalyst it is of no importance whether

5 a preliminary product of an artificial resin is soluble in pure water or not, but it must be soluble in the diluted alkali solution present at the addition of the catalyst. The textile material to be treated is impregnated with this dye bath and subjected to a heat treatment for the purpose of forming and hardening the final artificial resin.

A plurality of resins may be applied to the fibre, for instance by impregnating with a solution 10 containing both the original components for the formation of the one resin and the original components for the formation of another resin or a resin product.

It is surprising that the presence of the dye-stuff does not disturb the finishing operation and does not interfere with the finishing effects and that, moreover, the presence of artificial resin does not interfere with the dyeing, but on the contrary under certain conditions leads to dyeing effects of improved properties for instance with regard to genuineness.

The following examples show preferred modifications of the invention.

## Example 1

25 120 g. of dimethylol urea, 6 g. of ammonium sulphate, 14 g. o.o'-benzidine sulpho acid—2 grams nitro-m-phenylene di-amine are dissolved to 1000 cm<sup>3</sup> water, the textile material is impregnated with this solution, squeezed, dried and then heated to 130° C. to form the resin. A bright orange color and at the same time an excellent finishing effect result.

## Example 2

35 60 g. of dicyanogen-di-amide, 98 g. of 40 per cent formaldehyde solution, 10 g. of poly-vinyl alcohol, 6 g. of 1.3.8.naphthol-di-sulpho acid, 8 g. of cupric sulphate, 5 g. of tartaric acid are dissolved in 1000 cm<sup>3</sup> of water and treated as described in Example 1. A blue color results.

## Example 3

45 40 g. of phenol, 66 g. of formaldehyde, 8 g. of waste sulphite liquor, 6 g. of 25% ammonia solution, 4 g. of  $\beta$ -naphthol di-sulpho acid 2.6.8. are dissolved in 1000 cm<sup>3</sup> of water and treated as described in the preceding examples. A red color and at the same time excellent finishing effects, 50 as reduced swelling ability, etc., result.

## Example 4

55 A fabric treated in the manner usual in the textile industry with carbazole hydroxycarboxylic

acid arylide is dried and then subjected to a treatment in a bath of the following composition:  
To 1000 cm.<sup>3</sup> of water, 12 g. of 4-amino-1-benzoyl-amine-3-methoxy-6-methylbenzene, prepared by the usual diazotizing, 100 g. of urea, 140 g. of 40 per cent formaldehyde solution, 6 g. of acetic acid, 2 g. of ammonium phosphate. The textile material is impregnated with this solution and the dye-stuff is developed to a genuine dark blue with simultaneous applying of the substance forming the artificial resin. By a subsequent thermal maturing, the artificial resin is finally formed.

What we claim is:

In the method of dyeing and at the same time finishing textile materials, the steps of impregnating the material with carbazole hydroxycarboxylic acid arylide, then impregnating with an aqueous solution containing urea, formaldehyde, and diazotized 4-amino-1-benzoyl-amine-3-methoxy-6-methylbenzene, said latter solution being acid and containing a catalyst for the formation of the resin, and heat-treating said material for hardening of the artificial resin and fixation of the dyestuff.

ERNST SCHUBERT.  
HEINZ PIERER.